

July 18, 1944.

G. GAUTHIER

2,354,006

ALUMINUM BASE ALLOY WITH PROTECTIVE COATING

Filed Feb. 1, 1941

FIG. 1.



FIG. 2.



Inventor

Gaston Gauthier,

By *Alfred Lemoine*

Attorney.

## UNITED STATES PATENT OFFICE

2,354,006

ALUMINIUM BASE ALLOY WITH  
PROTECTIVE COATINGGaston Gauthier, Chambery, Savoie, France;  
vested in the Alien Property CustodianApplication February 1, 1941, Serial No. 377,049  
In France January 26, 1940

1 Claim. (Cl. 29—181)

For several years it has been endeavoured to use aluminium alloys containing at the same time magnesium, zinc, copper, nickel, and having the following compositions:

|    | Per cent                    |
|----|-----------------------------|
| Zn | Up to 15                    |
| Mg | Up to 7                     |
| Cu | Up to 5                     |
| Ni | Up to 3                     |
| Al | substantially the remainder |

Unfortunately, these alloys have a great tendency, even when they have been subjected to the most suitable heat treatments, cracking corrosion, or intercrystalline corrosion.

It has been endeavoured to remedy this inconvenience, either by refining the grain by addition of elements such as: Mn, Cr, Ti, V, Co, W, Mo, G1, Ce, or by any addition having, in particular, the effect of diminishing the corrodibility, for instance the elements Ca, Cd, Ag, Sb, Li.

By these additions, some of which have a favourable action on the characteristics, a very appreciable amelioration of the resistance to cracking corrosion has not in fact been obtained.

The applicant has noticed the surprising fact that a layer of plating, constituted by an aluminium alloy mainly containing zinc, ensured the protection; the zinc content must be higher than 0.5%.

Either in order to facilitate the intimate welding of the layer of plating with the alloy member to be protected, or to modify in a definite direction the diffusion between the layers of the alloy elements during the heat treatment, or for any other reason, a layer of metal or alloy, of different composition than that of both alloys, for instance a layer of aluminium of selected purity, may be interposed between the layer of plating and the foundation metal.

In the layer of aluminium-zinc alloy can advantageously be incorporated all the known elements for promoting the obtainment or the maintenance of a fine grain during the manufacture (melting, casting), heat treatments and mechanical distortions, such as small quantities of V, Ti, Zr, Mn, etc., together or separately but in total quantities smaller than 2%.

The elements entering into the composition of the protecting layer above defined could be the usual metals found on the market or, if a marked incorrodibility of the layer is to be ensured, use will be made of the purest metals, so-called "refined metals," that is to say of very low content in impurities, titrating more than 99.90%.

The plating layer of alloy of the above specified composition, can be plated on the ingots or members at any one of the phases of manufacture: It can be plated either before any transforming operation, or after the various transforming operations (extrusion, forging, rolling, etc.) or on the semi-finished products between certain transforming operations.

Referring to the drawing, Fig. 1 shows a sheet 10 of metal with the plating on one side and Fig. 2 with the plating on both sides.

The protection process applies not only to the manufacture of members obtained by mechanical transformation processes (extrusion, forging, 15 rolling, etc.) which utilise either ingots, or semi-finished products, but also applies to the case of foundry members, that is to say, to cast members used after more or less complex machining (fettling, drilling, milling, etc.).

20 The plating metal may be cast or welded to the foundation metal by any of the well known casting or welding processes.

The protecting alloy layer of the composition specified can also be secured by atomizing by a 25 known process said protecting metal either at the surface of a cast ingot adapted to be transformed by one of the known means (extrusion, forging, stamping, etc.), or at the surface of members adapted to be used such as they come from casting, or again, at the surface of blanks adapted to be subjected to a complementary transforming operation by a known process (extrusion, forging, rolling, etc.), or at the surface of finished members obtained by known processes (extrusion, 30 forging, rolling, etc.).

The protecting layer of the composition specified can also be produced by an electrolytic process, or by a chemical process such as surface precipitation or cementation, that is to say by a 35 modification of the composition of the superficial part of the ingot by the action of salts, metals, alloys, intermetallic compounds or mixtures of these various bodies. These modifications can be effected on the ingots, sand-cast or chill-cast members, finished or semi-finished products.

Said cementation can consist, as usual, in increasing the content of the cortical layer in certain elements (Zn, for instance), or in diminishing the content in certain other elements (Mg for instance), or by evaporation (eventually during the heat treatment), or by oxidation (by tempering in a bath which can be an oxidizing molten bath such as potassium bichromate), or 50 by any other reaction with a gaseous atmosphere,

a liquid or solid salt, an alloy, or a suitable mixture of these bodies.

The plated members, finished or semi-finished products obtained can be subjected to ameliorating heat treatments suited to the foundation alloy. The dissolving treatment could eventually be prolonged until nearly complete homogenization of the plating layer and the foundation metal, or of the plating layer, the intermediate layer and the foundation metal, or of the intermediate layer and of one of the two other layers, if necessary for ensuring the suitable cohesion of the layers one to the other, for instance in view of important plastic or nonplastic distortions to which the member thus treated is to be subsequently subjected; or again for increasing the average mechanical characteristics of the compound product.

Solely for giving an idea of the efficiency of the process as regards protection against corrosion, by way of example, the following experiment will be cited:

A sheet metal plate 1 mm. thick was prepared with an aluminium base alloy having the composition:

|    | Per cent |
|----|----------|
| Fe | 0.60     |
| Si | 0.60     |
| Mg | 3.20     |
| Cu | 1.90     |
| Zn | 5.20     |
| Ni | 0.70     |
| Ti | 0.20     |

It showed as characteristics, after quenching at 475° C. and annealing to 120° for 24 hours:

Tensile strength=55 kg./mm.<sup>2</sup>

Elongation=14.7%

After having been maintained in a salt mist for three months, the tensile strengths of the 40 various test pieces were very variable: between

25 and 40 kg./mm.<sup>2</sup> and the elongations became so small that it was impossible to measure them. Their micrographic examination shows that an important intercrystalline corrosion had taken place.

A sheet metal plate 1 mm. thick was prepared with the same alloy, but covered on both sides for about 5% of the thickness, with an aluminium alloy containing 3% of zinc. Treated in 10 the same conditions as above, this sheet metal plate showed the following characteristics:

Tensile strength=50 kg./mm.<sup>2</sup>

Elongation=15%

After being maintained for three months in a salt mist, one obtained:

Tensile strength=50 kg./mm.<sup>2</sup>

Elongation=13.5%

20 In his copending application Serial No. 377,048, filed on even date herewith, applicant discloses and claims the protection of an aluminium alloy which contains up to 15% zinc, up to 7% magnesium, up to 5% copper, up to 3% nickel and up to 2% chromium, by means of a layer of an aluminium-zinc alloy which contains more than 0.5% zinc.

I claim:

30 An aluminium base alloy, comprising a foundation member of the type that has a propensity to undergo cracking intercrystalline corrosion, containing a major significant quantity of zinc up to 15%, minor significant quantities of magnesium up to 7% and copper up to 5% and nickel up to 3%, respectively, an adherent coating thereon comprising an aluminium base alloy containing a minor quantity of zinc in an amount of the order of 0.5-3.0% but not less than 0.5%.

GASTON GAUTHIER.